

Oct. 6, 1931.

F. GREINER

1,826,211

PROCESS OF MANUFACTURING GRAY PIG IRON

Filed May 14, 1928



Inventor

Fritz Greiner

By Knights & Bow  
attys.

## UNITED STATES PATENT OFFICE

FRITZ GREINER, OF STUTTGART-CANNSTATT, GERMANY, ASSIGNOR TO MASCHINEN-FABRIK ESSLINGEN, OF ESSLINGEN, GERMANY

## PROCESS OF MANUFACTURING GRAY PIG IRON

Application filed May 14, 1928, Serial No. 277,746, and in Germany May 27, 1927.

My invention relates to a process of manufacturing gray iron castings of any desired structure having a low percentage of carbon and is an improvement on the process described in my copending application, Serial No. 146,801, filed November 6, 1926, now Patent No. 1,746,467. According to the process described in that application the desired physical properties and structure are obtained by controlling the composition of the mixture from which the castings are made in such a manner that the total content of C+Si is selected in accordance with the thickness of the walls of the article to be cast, the proportion of C+Si being increased as the wall thickness decreases, for producing any given structure.

For producing an iron with a low percentage of carbon which is frequently aimed at and especially desired at the present time, in view of the great tensile strength resulting therefrom and due to the decrease of the number and size of the graphite lamellæ, the method described in my said copending application does not suffice. For this reason in such cases according to my invention the percentage of the carbon is retained unaltered and only the amount of silicon contained in the iron is made to suit the varying conditions. The amount of silicon required with regard to the wall thickness can then be ascertained in a simple manner from a diagram owing to relations which by law exist between the wall thicknesses on the one hand and the amounts of carbon and silicon on the other hand.

Thus according to my invention the process consists therein that for the largest possible group of compositions of varying wall thicknesses and for different kinds of castings the percentage of carbon is maintained the same and that only the percentage of silicon is altered accordingly. This is preferably done with reference to a diagram as shown on the drawing in which the wall thicknesses are marked on the ordinates and the contents of silicon on the abscissæ. For a certain contents of carbon of for instance 3% the contents of silicon necessary for a definite wall thickness can then be taken from

a straight line the values of which increase as the wall thicknesses decrease. It is then still left at the discretion of the foundryman to decide upon the contents of carbon most favourable for the occasion. It is usually fixed at between 2.8 and 3%, as with such contents the iron possesses a great fluidity and also a very high tensile strength.

I claim as my invention:

1. The process of producing a gray iron casting of any desired structure which consists in first preparing a molten mixture of iron, carbon and silicon, the proportion of silicon being adjusted in accordance with a curve which rises substantially in a straight line as the wall thickness of the article to be cast decreases, the proportion of carbon being maintained substantially the same for all wall thicknesses, and then pouring said molten mixture into a mold.

2. The process of producing a gray iron casting of any desired structure which consists in first preparing a molten mixture of iron, carbon and silicon, the proportion of silicon being adjusted in accordance with a curve which rises substantially in a straight line from 0.8% to 2.8% as the wall thickness decreases from 50 mm. to 5 mm., the proportion of carbon being maintained at 3% for all wall thicknesses, and then pouring said molten mixture into a mold.

3. The process of producing a gray iron casting of a particular structure which consists in first preparing a molten mixture of iron, carbon and silicon, the carbon content being low and substantially the same for a large group of wall thicknesses of the articles to be cast and the silicon content being adjusted to the wall thickness in accordance with the diagram shown in the drawing, and then pouring the mixture into a mold.

In testimony whereof I affix my signature.  
FRITZ GREINER.